

## UNITED STATES PATENT OFFICE

2,083,982

## WEIGHTING TEXTILE MATERIALS

Herman S. Bosland, Paterson, N. J., assignor  
to Stein, Hall & Company, Inc., New York,  
N. Y., a corporation of New York

No Drawing. Application September 8, 1936,  
Serial No. 99,875

14 Claims. (Cl. 134—16)

This invention relates to the treatment of fibrous materials, more particularly textile materials, and to a new and improved method for finishing such materials. It especially relates to the weighting of textile fabrics.

In the treatment of materials such as cotton it is customary to subject the cloth to soap scouring, kier boiling, mercerizing, and bleaching prior to dyeing or printing. The bleaching and scouring action sometimes causes the cotton to lose 10% to 15%, or even 20%, of the natural gums and oils. To regain this weight the cotton has heretofore been treated with loading or weighting materials including metallic salts, such as magnesium sulphate, calcium chloride, or similar compounds, or sugar. Many objections have been raised to the use of such metallic salts and in some countries it is forbidden to import materials containing them. Sugar is objectionable because it caramelizes in the mechanical finishing processes of drying, ironing, steaming, pressing and the like. Moreover, sugar is also objectionable because it is too hygroscopic.

It is also common practice in the textile industry to add various substances to the fibers to make them pliable and soft, e. g., oils, fats, glycerine, and the like. Ordinary dextrins, thin-boiling starches and similar materials, if used to coat the fabrics produce a hard finish.

Both of the foregoing treatments are herein referred to generically as "finishing treatments" because they are applied at the last or finishing stage of manufacture.

It is to be observed, however, that there are a number of points of distinction between weighting and the various fulling and softening treatments. For instance, weighting is especially important in finishing textiles made from natural fibrous materials, such as cotton, which lose weight during the various processing steps. A fulling and softening treatment might be advantageous, however, on any type of textile material which tends to be stiff, including artificial as well as natural materials. In present practice, as will be apparent from the foregoing discussion, the weighting materials are quite different physically and chemically from the softening agents.

One of the objects of the present invention is to provide new and improved compositions for finishing textile materials in which the ingredients of the finishing composition are the same for weighting or softening, although usually different in proportions and concentrations. Another object is to provide compositions which produce both weighting and softening effects. A

further object is to produce fibrous materials containing new and improved finishing compositions. Another object is to provide a method of producing softening effects on textile materials without the use of sulfonated oils, glycerine, or other customary softening agents. Another object is to provide a method of weighting or finishing cotton materials with compositions which do not yield an ash content on burning and which are free from the objections inherent in the use of metallic salts, glucose, sugar and similar materials. Another object is to provide a new and improved method of finishing textile materials with the aid of amylaceous products. Other objects will appear as the description proceeds.

In accomplishing these objects in accordance with the invention, it has been found that new and improved results in the treatment of fibrous materials, more particularly in finishing, and especially in weighting, such materials, may be obtained by the use of compositions containing a water-dispersible, film-forming substance or binding agent, preferably a starch degeneration product, and urea. The mechanical steps may be the same as those now used in the art, and any other method may be used as long as the materials are suitably impregnated, immersed, or coated with a composition of the character described.

It will be recognized that the type of composition employed may vary, depending upon the desired results. For weighting it is preferable to employ a composition containing a major proportion of urea and a minor proportion of binding agent. The amount of the composition applied to the fibrous material will also vary depending upon the results desired, and in the case of a mere fulling or softening treatment will usually be relatively small, as, for instance, 4% to 6% by weight of the material, while in weighting it may be relatively large, for example, 20% to 40% by weight of the material.

The invention will be further illustrated, but is not limited, by the following examples, in which the quantities are stated in parts by weight:

*Example I*

A weighting composition was prepared by heating together a mixture of 50 parts of a modified starch, 50 parts of urea and 200 parts of water, to a temperature of about 180° to about 200° F. for 15 minutes.

A gingham material which had previously been scoured, kier boiled, mercerized and bleached in the usual manner for cotton material was then

passed through this finishing bath and dried. It was noted that the material had gained 38% in weight and a relatively stiff finish was obtained.

*Example II*

5 Twenty-five (25) parts of a modified starch were mixed with 75 parts of urea and 200 parts of water, and heated to 180° to 200° F. for 15 minutes.

10 A gingham material similar to that used in Example I was then immersed in this composition at a temperature around 140° to 150° F. and dried. It was noted that the material had gained 33% in weight, possessed a soft finish and a nice feel. 15 It was not soggy, as is often the case when similar material is finished with weighted gums containing glucose, sugar and the like, or metallic salts such as calcium chloride. No caramelization or browning effect was noted on drying, as 20 in the case where sugar compositions are used. When the material was burned no ash content due to the weighting composition was produced.

In a similar manner other compositions may be prepared in accordance with the invention, with 25 varying proportions of urea and amylaceous matter. It is usually preferable to employ a starch degeneration product, by which is meant a derivative of starch such as may be obtained by the various processes of making thin-boiling and so-called soluble starches and dextrans. In general, especially good results have been obtained with specially modified starches. By a specially modified starch is meant a starch degeneration product which, after having been colloidally dispersed 30 in water, yields a dried protective film of suitable physical characteristics for the purpose involved. In order to obtain these characteristics and to form so-called solutions suitable for textile application, ordinary undegenerated starch is suitably degenerated in part, or modified, by various 35 chemical and heat treatments.

If desired, mixtures of undegenerated starch and modified starches may be used in conjunction with the urea. While it is preferable to use a starch degeneration product, in some instances, 45 as, for example, in the treatment of cotton materials, ordinary starch may be used. The term "starch degeneration product" is herein employed to cover dextrans as well as modified starches. 50 Among the suitable starchy materials may be mentioned wheat, rye, barley, oat, rice, maize and potato starches, sago and cassava flours, and colloidal modifications thereof, and other starches and flours and derivatives thereof.

55 As previously indicated, the proportions and concentrations of materials may vary depending upon the type of material treated, and upon other related factors. In the compositions of the invention the ratio of solids to water is preferably greater than 1:4 and very good results have been 60 obtained in weighting with a ratio of solids to water of about 1:2.

The amount of urea will be determined to some extent by the amount of water because the maximum amount of urea will normally be less than the amount required for saturation under ordinary temperature and pressure conditions. In 65 weighting textile materials, it has been noted that the use of major amounts of urea and minor amounts of binding agents normally gives softer and more pliable materials than equal amounts of urea and binding agent, or smaller amounts of urea and larger amounts of binding agent. (Cf. Examples I and II.)

75 The amount of the composition retained by the

material treated will depend largely upon the concentration of the bath and the time of treatment. Ordinarily the bath may be either hot or cold, but in some instances it is desirable to use a relatively warm bath.

It will be recognized that a wide variety of auxiliary agents may be added to the compositions herein described. Among such addition agents may be mentioned fuller's earth, bentonite, wetting, penetrating and dispersing agents, 10 for example, sulfonated oils, higher alcohol sulfates (e. g., dodecyl sulfate, cetyl sulfate, and similar compounds), diethylene glycol, glycerine and related substances. The proportions of these materials may also vary, depending upon the type 15 of treatment and the material treated.

In preparing the various compositions, it is preferable to prepare a dry blend of binding agent and urea as a base material. This blend is marketed in dry or powdered form and requires 20 only the addition of water, and mixing, preferably with heating, to produce the composition in dispersed form. Auxiliary materials may also be included in the dry base.

The type of material treated is subject to variation, but ordinarily any textile material, and particularly woven materials may be treated in accordance with the invention. Among the materials which may be given a finishing treatment as herein described are cloth, fabrics or 25 flexible sheet materials made from cotton, linen, wool, asbestos, glass yarn, cellulose esters and ethers, and regenerated cellulose prepared in any suitable manner, e. g., by the viscose, nitration and cuprammonium methods. It will be recognized that the weighting treatment applies particularly to cotton and materials which lose their natural oils and waxes in processing.

The use of a binding agent, and especially a 30 starchy material, in conjunction with urea in finishing fibrous materials, has many advantages over the use of the binding agent or urea per se. Thus, it has been proposed to finish textile materials by a treatment with urea solutions and thereby to reduce the inflammability of the material. 35 It has also been proposed to use urea as well as a large number of other organic compounds as swelling agents for cellulose acetate to render it more absorptive to dyes. However, the use of urea alone does not fulfill the functions of the 40 combination of urea and starch or starch degeneration products. Better fulling and softening effects are obtained by this invention and, in weighting, by the use of suitable proportions of 45 urea and binding agent, it is possible to produce a relatively large increase in weight without destroying the softness, fullness and pliability of the 50 fabric.

While it has heretofore been proposed to produce softening effects by using substances such 55 as sulfonated oil, glycerine and the like, insofar as is known, the use of, and the advantage of using, urea in conjunction with binding agents has not heretofore been suggested. It may be noted that urea has the special advantage over sulfonated 60 oils and similar substances in that it is essentially a dry solid and the finishing compositions may be marketed as a dry base requiring no further addition of auxiliary agents other than water.

Having thus described the invention, what I 70 claim as new and desire to secure by Letters Patent of the United States is:

1. A textile weighting composition consisting of an intimate dispersion of an amylaceous substance, urea and water, the amount of urea being 75

- at least equal by weight to the amount of amy-  
laceous substance.
2. A textile weighting composition consisting  
of a major proportion by weight of urea and a  
5 minor proportion by weight of amylaceous sub-  
stance.
3. A textile weighting composition consisting of  
an intimate dispersion of about twenty-five to  
about fifty parts by weight of a starch degenera-  
10 tion product and about fifty to about seventy-  
five parts by weight of urea in about two hun-  
dred parts by weight of water.
4. A textile weighting composition consisting of  
an intimate dispersion of a dextrin, urea and  
15 water, the amount of urea by weight being at  
least equal to the amount of dextrin.
5. A textile weighting composition consisting of  
an intimate dispersion of a dextrin, urea and  
20 water in which the amount of urea by weight is  
substantially greater than the amount of dextrin.
6. A textile weighting composition consisting of  
an intimate dispersion of a modified starch and  
urea, the ratio of modified starch and urea vary-  
25 ing from about twenty-five to about fifty parts  
of modified starch to about fifty to seventy-five  
parts of urea.
7. A textile material weighted and finished with  
an intimate dispersion consisting of an amyla-  
ceous substance and urea, the amount of urea  
30 being at least equal to the amount by weight of  
the amylaceous substance.
8. A weighting composition consisting of an  
intimate dispersion of a starch degeneration  
product and urea in water, the amount of urea  
35 being at least equal to the amount of the de-  
generated starch, and the amount of water cor-  
responding to a ratio of solids to water by weight  
within the range of about 1:2 to about 1:4.
9. A weighting and finishing composition com-  
40 prising urea and amylaceous material in the ratio  
of approximately 3:1, said amylaceous material  
being the sole or substantially the sole binding  
constituent of the composition.
10. A weighting or finishing composition hav-  
ing an amylaceous material as its sole or sub-  
stantially its sole binding constituent, said com-  
position containing urea in an amount at least  
equal by weight to the amount of amylaceous  
material.
11. A textile weighting and finishing composi-  
10 tion having an amylaceous material as its sole or  
substantially its sole binding constituent, said  
composition containing urea in an amount in ex-  
cess of the amount of amylaceous material.
12. The method of weighting cotton cloth from  
15 which at least a portion of the natural oils has  
been removed by previous processing treatments  
which comprises applying thereto a composition  
having an amylaceous material as its sole or sub-  
stantially its sole binding constituent, said com-  
position containing urea in an amount at least  
20 equal by weight to the amount of amylaceous  
material.
13. The method of weighting cotton cloth from  
which at least a portion of the natural oils has  
25 been removed by previous processing treatments,  
which comprises applying thereto an intimate  
dispersion consisting of an amylaceous substance  
and urea in water, the amount of urea being at  
least equal to the amount of amylaceous sub-  
30 stance and the ratio of solids to water being with-  
in the range of about 1:2 to about 1:4.
14. A textile material weighted and finished  
with a composition having an amylaceous ma-  
35 terial as its sole or substantially its sole binding  
constituent, said composition containing urea in  
an amount at least equal by weight to the amount  
of amylaceous material.

HERMAN S. BOSLAND. 40